

## UNITED STATES PATENT OFFICE

2,575,026

IMPROVING FASTNESS TO CROCKING OF  
AZOIC DYED MATERIALS USING CERTAIN  
VINYL RESINSElmer H. Rossin, Melrose, Mass., assignor to Mon-  
santo Chemical Company, St. Louis, Mo., a cor-  
poration of DelawareNo Drawing. Application May 28, 1948;  
Serial No. 29,923

12 Claims. (Cl. 8—18)

1

The present invention relates to a method of improving the fastness to crocking or rub-off of azoic dyed or naphthol dyed cotton textile and other similarly dyed cellulosic materials.

Azoic dyes or naphthol colors, which terms are used interchangeably hereinafter, generally have excellent wash-fastness and light-fastness and are generally considered to be on a par with vat dyes in this respect. In addition, azoic dyes have an economic advantage over vat dyes when either may be used for a particular dyeing job. However, azoic dyed fabrics have one disadvantage which has not been satisfactorily overcome in the past, namely, the crocking or rubbing off of the dye from the surface of the dyed fabric. A number of techniques have been developed which tend to lessen the degree of crocking of such dyes, but none have been successful heretofore, and for this and other reasons the widespread use of azoic dyes has been materially curtailed.

The present invention provides a simple and efficient method for overcoming the aforementioned difficulties and permits the widespread use of azoic dyes for dyeing all types of cellulosic fabrics and other cellulosic materials, and also other materials which may be dyed with azoic dyes. The present invention also provides an azoic dyed cellulosic material which is substantially fast to crocking even after a considerable number of launderings.

It is, accordingly, one object of the present invention to provide a method of improving the fastness to crocking of azoic dyed cellulosic textiles and other cellulosic materials.

A further object of the invention is to provide an azoic dyed cotton or other cellulosic material which is substantially fast to crocking and which retains its fastness to crocking after a number of cotton washes or launderings.

Other objects and advantages of the invention will appear from the following description and the appended claims.

These and other objects are, in general, attained by first impregnating the cotton textile such as a fabric or yarn, or other cellulosic material, with a naphthol developing agent such as  $\beta$ -naphthol, certain derivatives of  $\beta$ -hydroxy naphthoic acid and the like and then coupling the developer in situ on the cotton textile or other cellulosic material with a diazotized base or salt

2

as, for example, Fast Scarlet Salt RN (color index 118) to form an azoic dyed material. The cotton textile or other cellulosic material is then impregnated with an aqueous solution comprising a relatively small proportion of a water-soluble or water-dispersible ammonium, amine or amidated salt or derivative of a copolymer of a polymerizable vinyl compound having the structural formula R—CH=CH<sub>2</sub>, where R is a phenyl or substituted phenyl radical with an ethylene  $\alpha,\beta$ -dicarboxylic anhydride or acid, or alkyl half ester of such acid, in which the alkyl group contains from 1 to 6 carbon atoms or mixtures thereof; and is then dried, preferably at elevated temperatures, to insolubilize the copolymeric salt or derivative.

The foregoing method possesses several advantages over prior methods of dyeing with azoic dyes in that the cotton or other cellulosic material need not be dried after the developer has been applied as is customarily done, nor is it necessary to soap and rinse such material after the developer and diazotized salt or base have been coupled in situ. However, either or both of these customary procedures may be used if desired. The omission of the drying step in the manner indicated is of particular importance since it is well known that a duller shade is obtained when the material is dried after the developer has been applied.

Suitable ammonium or amine salts or amidated derivatives of the foregoing copolymers which may be employed in the practice of the invention include the salts of ammonia or an amine as, for example, methyl, ethyl, propyl, butyl amine and the like. Other water-soluble amine or amidated derivatives of such copolymers will be apparent to those skilled in the art. Of the salts and derivatives aforementioned, the ammonium salt is preferred.

The fastness to crocking of the azoic dyed material, prepared as described above, is, in general, made substantially permanent by heating the fabric or material to a temperature of about 230° F. to 325° F., a temperature of about 230 to 260° F. being preferred. However, a good permanent effect may be obtained by heating the treated fabric at temperatures of 180° to 230° F. In the latter case good fastness to crocking will still be apparent after a number of launderings or cotton washes. Excellent fastness to crocking, which

fastness is substantially permanent for the normal life of the material, may also be attained by incorporating in the aqueous solution containing the above described copolymeric salts a small proportion of a compound which possesses pre-reactivity for carboxyl groups, such as a thermosetting resin, for example, a phenol-formaldehyde resin or an amino-formaldehyde resin such as melamine-formaldehyde resins, urea-formaldehyde resins and the like. In place of such resins, formaldehyde or materials which yield formaldehyde at the temperature above indicated or alkylene polyamines such as ethylene diamines, propylene diamines, butylene diamines, diethylene triamine and the like may be used. The quantities of such thermosetting resin formaldehyde or polyamine which can be used may be varied to some extent, but, in general, such materials are employed in quantities varying between about 5 to 20% by weight based on said copolymeric salt.

The copolymers which are employed in the present invention may be prepared in various ways. In general, they are prepared by copolymerizing an ethylene  $\alpha,\beta$ -dicarboxylic acid or anhydride such as maleic acid, fumaric acid, maleic anhydride and the like, or preformed alkyl half esters of such acids in which the alkyl groups contain from 1 to 6 carbon atoms or mixtures of such acids, anhydrides or esters, with a polymerizable vinyl compound having the structural formula  $R-CH=CH_2$ , where R is a phenyl radical, a halogen substituted phenyl radical such as chloro-phenyl dichloro-phenyl and the like or a methyl substituted phenyl radical such as methyl phenyl, dimethyl phenyl and the like or mixtures thereof. In general, the above described dicarboxylic components and vinyl compounds are copolymerized in a molal ratio varying between about 1:1 to 1:2, and preferably in a molal ratio varying between about 1:1.1 to 1:1.5. Of the above described copolymerizable components, styrene and maleic anhydride, or styrene and mixtures of maleic anhydride and alkyl half esters of maleic acid, in which the alkyl group contains from 1 to 4 carbon atoms, are preferably employed in the preparation of such copolymer.

When alkyl half esters of ethylene  $\alpha,\beta$ -dicarboxylic acids or anhydrides are employed as indicated, they are in general prepared by reacting an appropriate alcohol having from 1 to 6, and preferably 1 to 4, carbon atoms, such as methanol, ethanol and the like with such acid or anhydride in a molal ratio varying between about 1:1 to 1:2.

A variety of copolymerization methods may be used depending upon the mutual solubility or non-solubility of the above described polymerizable components. In the case of styrene and maleic anhydride, for example, the well-known mass polymerization may be used since these monomers are mutually soluble. In this method the monomers are copolymerized by heating them at temperatures varying between about 100° to 300° F. for a period of several hours, if desired, in the presence of a polymerization catalyst such as a peroxide catalyst, for example, benzoyl peroxide.

Emulsion polymerization methods may be used or the monomers may be copolymerized in a non-reactive solvent such as xylene, which is a solvent for certain of the above monomers, but is a non-solvent for the copolymer. The temperature of the reactants is generally maintained at the boiling point of the solvent. The copolymer, which precipitates as it is formed, is separated

from the liquid phase by centrifuging, filtration and the like.

The ammonia or amine salt of the copolymer is prepared, for example, by adding the copolymer to an aqueous solution containing a quantity of ammonia, amine and the like sufficient to yield a solution of the copolymer in water. The solution obtained is not necessarily a true solution and in most instances will probably be a colloidal solution.

A further understanding of the invention will be obtained from the following illustrative examples, parts being by weight.

*Example I*

A wax-free, clean cotton fabric was padded through a long bath (10 parts liquid to 1 part fabric) comprising a naphthol developer. This bath was made up as follows:

|                                                                            | Parts |
|----------------------------------------------------------------------------|-------|
| Naphthol AS ( $\beta$ -hydroxy naphthoic acid anhydride)                   | 10    |
| Ethanol                                                                    | 12    |
| Water                                                                      | 10    |
| 25 NaOH (as an aqueous solution containing 330 parts NaOH/950 parts water) | 4     |
| Formaldehyde (37%)                                                         | 30    |

The above NaOH solution was added until the solution turned clear brown. The above ingredients were then added to 1000 parts of water to which had been added 2 parts of a 30% solution of sodium dodecyl benzene sulfonate in water and 13.5 parts of 38° Bé. NaOH solution. The bath was maintained at about 70-80° C. during the padding operation and the pick-up was such as to put on a quantity of liquid substantially equal to the dry fabric weight.

The fabric comprising the developer was then padded through a long bath (10-1) comprising a diazotized salt which coupled with the developer in situ on the fabric. This bath had the following composition:

|                                        | Parts |
|----------------------------------------|-------|
| Water                                  | 990   |
| Sodium chloride                        | 20    |
| Fast Scarlet Salt RN (color index 118) | 15    |

This solution was maintained at about 60° F. after preparation and during the padding operation. The pad rolls were adjusted so as to obtain about 100% pick-up.

The dyed fabric was then padded through a solution containing two parts of the ammonium salt of the copolymer prepared as described below per 98 parts of water. This solution was maintained at about 125° F. during the padding operation and the pad rolls were adjusted so as to obtain a 100% pick-up of the solution.

After the fabric had been treated by the above procedure, it was dried at a temperature of 250° F. The finished fabric which possessed a bright red shade, had a slightly stiffened hand and excellent fastness to crocking. The fabric was boiled in a solution containing 2% sodium dodecyl benzene sulfonate for one hour without any appreciable red coloration of the solution and on drying was substantially fast to crocking. The fabric was then given three standard AATCC cotton washes and its fastness to crocking was not appreciably affected thereby.

The ammonium salt of the copolymer employed as described above was prepared by first reacting 0.2 molecular proportions of methanol with 1 molecular proportion of maleic anhydride at a temperature of about 75° C. until the reac-

tion product had a substantially constant acid value on continued heating. The resulting mixture was then copolymerized with about 1.04 molecular proportions of styrene by heating the mass to a temperature of about 80° C. and maintaining this temperature during the period of rapid heat evolution, after which the temperature was raised to 120° C. to complete the reaction. The hard, glassy resin, which was obtained on cooling the reactants, was then comminuted to make it more readily soluble. Two hundred parts of this copolymer were dissolved in an aqueous solution made up of 2500 parts of water and 132 parts of 26° Bé. ammonia solution. This solution was then diluted with 8080 parts of water to form a solution containing approximately 2 parts of the ammonia salt of the copolymer per 98 parts of water (as employed above).

### Example II

A skein of wax-free, clean 10's cotton yarn was immersed in a long bath (10 parts liquid to 1 part fabric) comprising a naphthol developer. This bath was made up by first mixing 10 parts of naphthol As, 12 parts of ethanol and 10 parts of water and then adding an aqueous sodium hydroxide solution (containing 330 parts NaOH per 950 parts of water) until the solution turned clear brown. Thirty parts of 37% formaldehyde were then added to the above ingredients and the whole was added to 1000 parts of water to which had been added 2 parts of a 30% solution of sodium dodecyl benzene sulfonate in water and 13.5 parts of 38° Bé. NaOH solution. The resulting bath was maintained at 80° C. during the impregnating operation. The skein was run through a wringer after immersion in the bath.

The skein comprising the developer was then immersed for about 2 minutes in a long bath (10-1) containing 20 parts of sodium chloride and 15 parts of Fast Scarlet Salt RN (color index 118) per 990 parts of water. This bath was maintained at about 50° F. after preparation and during the immersion of the skein therein. Excess bath was removed by running the skein through a conventional wringing device.

The skein of dyed yarn was then immersed for two minutes in a solution prepared by first dissolving 200 parts of the comminuted resin or copolymer, as prepared in Example I, in 2500 parts of water to which had been added 132 parts of 26° Bé. ammonia solution and then diluting this solution with 5070 parts of water containing 25 parts of formaldehyde. This solution was maintained at 70° F. during the immersion of the skein therein. The skein was then passed through a wringer to remove excess solution and was then dried at about 180° F. for a period of several hours. The dyed yarn which had a bright red shade possessed excellent fastness to crocking and retained this property after soaping for 1 hour at the boil in a 2% soap solution and drying. Moreover, the soap solution was substantially free of red coloration during the soaping operation. The dyed yarn possessed excellent fastness to crocking after 3 standard AATCC cotton washes.

### Example III

2 # packages of 12's cotton yarn wound on coiled spring cores were treated on a Franklin Package Machine using a long bath (10-1) containing a developer. This bath was prepared as described in Examples I and II and maintained at about 70° C. during the package treatment.

The circulation of the bath through the packages was as follows (using 5 lbs. gauge pressure):

|   | Minutes                               |
|---|---------------------------------------|
| 5 | Inside of package toward outside..... |
|   | 5                                     |
|   | Outside of package toward inside..... |
|   | 5                                     |
|   | Inside of package toward outside..... |
|   | 10                                    |
|   | Outside of package toward inside..... |
|   | 10                                    |

The packages were then treated with a long bath (10-1) containing 20 parts of sodium chloride and 15 parts of Fast Scarlet Salt RN (color index 118) per 990 parts of water. This bath was maintained at about 65° F. during the treatment. The bath was circulated through the packages from inside to outside and outside to inside using the same schedule as given above.

The packages were next treated with the solution of the ammonium salt of the copolymer prepared as described in Example I (about 2

20 parts of the ammonium salt of the copolymer per 98 parts of water). This solution was maintained at about 125° F. and was circulated through the packages using the same schedule as was used with the bath containing the developer.

25 The packages were hydro-extracted for 2 minutes, dried at 180° F. and then heated for about 10 minutes at 260° F. The dyed yarn which had a bright red shade possessed excellent resistance to crocking and retained this property after 3 washes with boiling 3% soap solution, each wash being of 1 hour duration. This dyed yarn, when beamed, can be woven directly into a fabric without any further treatment.

The foregoing conditions such as temperatures, strengths of solution of the developer, diazotized salt and copolymer, pressure and circulation employed in package treatment, duration of dyeing and treatment with the copolymeric salt, and other conditions may be varied considerably in carrying out the practice of the invention as will be apparent to those skilled in the art. Specifically, however, it is preferred to employ an aqueous solution of the copolymeric salt of the type hereinbefore described in which such copolymeric salt is present in amounts ranging from about 0.5 to 5.0% by weight. The quantity of copolymeric salt actually deposited on the fabric or yarn will vary depending upon the amount, for example, that is picked up by padding or

50 the extent to which the yarn or fabric is extracted, wrung, centrifuged or the like. In general, from 0.4 to 5.0% by weight of the copolymeric salt is deposited on the fabric, yarn or the material which has been dyed, based on the weight of such material.

Cellulosic materials other than cotton fabrics and yarns can also be dyed with azoic dyes and rendered fast to crocking by the method described herein. As examples of such materials may be 60 mentioned fabrics and yarns fabricated from jute, flax, linen, viscose rayon, cuprammonium rayon and the like or fabrics made from a combination of yarns fabricated from such materials. Other cellulosic materials can also be treated by the process or method described herein, if desired.

Instead of forming azoic dyes or naphthol colors in situ on cellulosic materials by the procedure hereinbefore described, other techniques may be used to apply such dyes in situ to fabrics or yarns. Moreover, other combinations of naphthol developer and diazotized salt or base may be used depending upon the shade, light-fastness, wash-fastness and the like which is desired. Examples of such combinations which are produced by the coupling of

a naphthol developer with a diazo-salt or base and are suitable for making azoic dyes appear in the following table:

| Naphthol Developer                                                      | Diazo Salt or Base                    |
|-------------------------------------------------------------------------|---------------------------------------|
| Naphthol AS ( $\beta$ -hydroxy naphthoic acid anilide).                 | Fast Garnet B Base (color index 82).  |
| $\beta$ -Naphthol.                                                      | Do.                                   |
| Naphthanol AS-D ( $\beta$ -hydroxy naphthoic acid o-toluidide).         | Do.                                   |
| Naphthanol BS ( $\beta$ -hydroxy naphthoic acid m-nitroanilide).        | Do.                                   |
| Naphthanol BS ( $\beta$ -hydroxy naphthoic acid $\alpha$ -naphthalide). | Do.                                   |
| Naphthanol MX ( $\beta$ -hydroxy naphthoic acid m-xylide).              | Do.                                   |
| Naphthanol OL ( $\beta$ -hydroxy naphthoic acid o-aniside).             | Do.                                   |
| Naphthanol OP ( $\beta$ -hydroxy naphthoic acid o-phenetide).           | Do.                                   |
| Naphthanol RL ( $\beta$ -hydroxy naphthoic acid p-aniside).             | Do.                                   |
| Naphthanol SW ( $\beta$ -hydroxy naphthoic acid $\beta$ -naphthilide).  | Do.                                   |
| Any of the above developers.                                            | Fast Orange R Base (color index 38).  |
| Do.                                                                     | Fast Scarlet G Base (color index 68). |
| Do.                                                                     | Fast Scarlet R Base (color index 69). |
| Naphthol AS.                                                            | diazotized m-nitro-p-toluidene.       |
| Any of the above developers.                                            | Fast Red BB Base (color index 113).   |
| $\beta$ -Naphthol.                                                      | Blue Red O Base (color index 123).    |
| Do.                                                                     | G Base (color index 258).             |
| Any of the above developers.                                            | Fast Blue B Salt (color index 499).   |
| Naphthanol SW.                                                          | Azo Black O Base (color index 500).   |

In addition to the combinations described in the above table, other combinations may be used as will be apparent to those skilled in the art. The color index referred to above is that published by the Society of Dyers and Colourists, edited by F. M. Rowe, 1st edition (1924).

Other means or procedures of dyeing fabrics or yarns with azoic dyes may be used in addition to those which have been described. For example, fabrics may be dyed in various types of apparatus by applying the developer first followed by coupling in situ with the diazo salt or base, or the developer and diazo salt or base in stabilized form may be applied to the fabric simultaneously. Moreover, yarns may be dyed on a beam or dyed as a running thread or by other procedures. The above described copolymeric salts may also be applied to fabrics, cotton raw stock, yarn and the like by the use of various types of equipment and by various modes of application.

The process described herein may also be employed to render fabrics, which have been printed with azoic dyes, substantially fast to crocking. The fabric may be printed by applying the developer and diazo salt or base, respectively, either successively or simultaneously. After the fabric has been printed with the azoic dye, it may be top printed with an aqueous solution of the copolymeric salt or such solution may be applied to the printed fabric in other ways.

Still further modifications of the process described herein will be apparent to those skilled in the art.

What is claimed is:

1. A process of improving the fastness to crocking of azoic dyed cellulosic materials which comprises first forming an azoic dye in situ on a cellulosic textile material selected from the group consisting of natural and regenerated cellulose textile materials by treating said material with a naphthol developer and a coupling agent selected from the group consisting of diazo salts and bases, subsequently treating said material with an aqueous solution comprising from 0.5 to 5% by weight of a water-soluble salt of a copolymer of 1 to 2 molecular proportions of a polymerizable vinyl compound having the structural formula  $R-CH=CH_2$ , where R is selected from the group consisting of the phenyl radical, a halogen substituted phenyl radical and a methyl substituted phenyl radical, with 1 molecular proportion of an ethylene  $\alpha,\beta$ -dicarboxylic compound selected from the group consisting of maleic anhydride, maleic acid, fumaric acid and alkyl half esters of said acids, in which the alkyl group contains from 1 to 6 carbon atoms, and mixtures of these compounds, said salt being selected from the group consisting of ammonium and amine salts, said solution being supplied in an amount sufficient to provide from about 0.4 to 5% by weight of said salt based on the weight of the material; and drying said material at temperatures above about 180° F. to substantially insolubilize said salt.

2. A process of improving the fastness to crocking of azoic dyed cellulosic materials which comprises first forming an azoic dye in situ on a cellulosic textile material selected from the group consisting of natural and regenerated cellulose textile materials by treating said material successively with a naphthol developer and a coupling agent selected from the group consisting of diazo salts and bases; subsequently treating said

material with an aqueous solution comprising from 0.5 to 5% by weight of a water-soluble copolymer of 1 to 2 molecular proportions of styrene with 1 molecular proportion of an ethylene  $\alpha,\beta$ -dicarboxylic compound selected from the group consisting of maleic anhydride, maleic acid, fumaric acid and alkyl half esters of said acids, in which the alkyl group contains from 1 to 6 carbon atoms, and mixtures of these compounds, said salt being selected from the group consisting of ammonium and amine salts, said solution being supplied in an amount sufficient to provide from about 0.4 to 5% by weight of said salt based on the weight of the material; and drying said material at temperatures above about 180° F. for a period of time sufficient to substantially insolubilize said salt.

3. A process of improving the fastness to crocking of azoic dyed cotton textile materials, fabric or yarn which comprises first forming an azoic dye in situ on a cotton textile material by treating same successively with a naphthol developer and a coupling agent selected from the group consisting of diazo salts and bases; subsequently treating said material with an aqueous solution comprising from 0.5 to 5% by weight of a water-soluble ammonium salt of a copolymer of 1 to 2 molecular proportions of styrene with 1 molecular proportion of a mixture of maleic anhydride and an alkyl half ester of maleic acid, in which the alkyl group contains from 1 to 4 carbon atoms, said solution being supplied in an amount sufficient to provide from about 0.4 to 5% by weight of said salt based on the weight of the material; and drying said material at temperatures above about 230° F. for a period of time sufficient to substantially insolubilize said ammonium salt.

4. A process of improving the fastness to crocking of azoic dyed cotton textile materials which comprises first forming an azoic dye in situ on a cotton textile material by treating same successively with a naphthol developer and a coupling agent selected from the group consisting of diazo salts and bases; subsequently treating said material with an aqueous solution comprising

75

from about 0.5 to 5% by weight of a water-soluble ammonium salt of a copolymer of 1 to 2 molecular proportions of styrene with 1 molecular proportion of a mixture of maleic anhydride and methyl acid maleate, said solution being supplied in an amount sufficient to provide from about 0.4 to 5% by weight of said salt based on the weight of the material; and drying said material at a temperature above about 230° F. for a period of time sufficient to substantially insolubilize said ammonium salt.

5. A process substantially according to *claim 4*, wherein the ammonium salt is the ammonium salt of a copolymer of 1 to 2 molecular proportions of styrene with 1 molecular proportion of a mixture of maleic anhydride and ethyl acid maleate.

6. A process substantially according to *claim 4*, wherein the ammonium salt is the ammonium salt of a copolymer of 1 to 2 molecular proportions of styrene with 1 molecular proportion of a mixture of maleic anhydride and propyl acid maleate.

7. A process of improving the fastness to crocking of azoic dyed cotton textile materials which comprises first forming an azoic dye in situ on a cotton textile material by treating the material successively with a naphthol developer and a coupling agent selected from the group consisting of diazo salts and bases; subsequently treating said material with an aqueous solution comprising from about 0.5 to 5% by weight of a water-soluble salt of a copolymer of 1 to 2 molecular proportions of a polymerizable vinyl compound having the structural formula  $R-\text{CH}=\text{CH}_2$ , where R is selected from the group consisting of the phenyl radical, a halogen substituted phenyl radical and a methyl substituted phenyl radical, with 1 molecular proportion of an ethylene  $\alpha,\beta$ -dicarboxylic compound selected from the group consisting of maleic anhydride, maleic acid, fumaric acid and alkyl half esters of said acids, in which the alkyl group contains from 1 to 6 carbon atoms, and mixtures of these compounds, said salt being selected from the group consisting of ammonium salts and amine salts, and from about 5 to 20%, based on said salt, of a substance selected from the group consisting of thermosetting resins, formaldehyde and alkylene polyamines, said solution being supplied in an amount sufficient to provide from about 0.4 to 5% by weight of said salt based on the weight of the material and drying said material at a temperature between about 230 and 325° F. for a period of time sufficient to insolubilize said salt.

8. A process substantially according to *claim 7* wherein said substance is a urea-formaldehyde thermosetting resin.

9. A process substantially according to *claim 7* wherein said substance is formaldehyde.

10. A process substantially according to *claim 7* wherein said substance is diethylene triamine.

11. An azoic dyed cellulosic textile material characterized by fastness to crocking, prepared by treating a cellulosic textile material selected from the group consisting of natural and regenerated cellulose textile materials with a naphthol developer and a coupling agent selected from the group consisting of diazo salts and bases, subsequently treating said material with an aqueous solution comprising from 0.5 to 5% by weight

of a water-soluble salt of a copolymer of 1 to 2 molecular proportions of a polymerizable vinyl compound having the structural formula  $R-\text{CH}=\text{CH}_2$  where R is selected from the group consisting of the phenyl radical, a halogen substituted phenyl radical and a methyl substituted phenyl radical, with 1 molecular proportion of an ethylene  $\alpha,\beta$ -dicarboxylic compound selected from the group consisting of maleic anhydride, maleic acid, fumaric acid and alkyl half esters of said acids, in which the alkyl group contains from 1 to 6 carbon atoms, and mixtures of these compounds, said salt being selected from the group consisting of ammonium salts and amine salts, said solution being supplied in an amount sufficient to provide from about 0.4 to 5% by weight of said salt based on the weight of the material; and drying said material at temperatures above about 180° F. to substantially insolubilize said salt.

12. An azoic dyed cellulosic textile material characterized by fastness to crocking, prepared by successively treating a cellulosic textile material selected from the group consisting of natural and regenerated cellulose textile materials with a naphthol developer and a coupling agent selected from the group consisting of diazo salts and bases, subsequently treating said material with an aqueous solution comprising (1) from 0.5 to 5% by weight of a water-soluble salt of a copolymer of 1 to 2 molecular proportions of a polymerizable vinyl compound having the structural formula  $R-\text{CH}=\text{CH}_2$ , where R is selected from the group consisting of the phenyl radical, a halogen substituted phenyl radical and a methyl substituted phenyl radical, with 1 molecular proportion of an ethylene  $\alpha,\beta$ -dicarboxylic compound selected from the group consisting of maleic anhydride, maleic acid, fumaric acid and alkyl half esters of said acids, in which the alkyl group contains from 1 to 6 carbon atoms, and mixtures of these compounds, said salt being selected from the group consisting of ammonium and amine salts and (2) a substance selected from the group consisting of thermosetting resins, formaldehyde and alkylene polyamines, said solution being supplied in an amount sufficient to provide from about 0.4 to 5% by weight of said salt based on the weight of the material; and drying said material at temperatures above about 180° F. to insolubilize said salt.

ELMER H. ROSSIN.

#### REFERENCES CITED

55 The following references are of record in the file of this patent:

#### UNITED STATES PATENTS

| Number    | Name            | Date          |
|-----------|-----------------|---------------|
| 2,047,398 | Voss -----      | July 14, 1936 |
| 2,322,333 | Widmer -----    | June 22, 1943 |
| 2,356,879 | Pense -----     | Aug. 29, 1944 |
| 2,416,884 | Schreiber ----- | Mar. 4, 1947  |

#### OTHER REFERENCES

- 65 Silk Hour. and Rayon World for October 1947, pp. 46, 48, 51. 8-18.  
 Am. Dyestuff Reporter for April 22, 1946, p. P197. 8-55.  
 Ser. No. 397,138, Fikentscher (A. P. C.), published May 11, 1943.